

Feb. 12, 1963

P. BUDININKAS

3,077,285

TIN-NICKEL-PHOSPHORUS ALLOY COATINGS

Filed Sept. 15, 1961

6 Sheets-Sheet 1

FIG. 1



FIG. 2



FIG. 3



FIG. 4



INVENTOR.

Pranas Budininkas

BY

Prangley, Baird, Clayton,  
Miller & Vogel, Attnys.

Feb. 12, 1963

P. BUDININKAS

3,077,285

TIN-NICKEL-PHOSPHORUS ALLOY COATINGS

Filed Sept. 15, 1961

6 Sheets-Sheet 2



Feb. 12, 1963

P. BUDININKAS

3,077,285

TIN-NICKEL-PHOSPHORUS ALLOY COATINGS

Filed Sept. 15, 1961

6 Sheets-Sheet 3



FIG. 6



FIG. 7

INVENTOR.  
Pranas Budininkas

BY

Prangley, Baird, Clayton,  
Miller & Vogel, Attys.

Feb. 12, 1963

P. BUDININKAS

**3,077,285**

## TIN-NICKEL-PHOSPHORUS ALLOY COATINGS

Filed Sept. 15, 1961

6 Sheets-Sheet 4



*INVENTOR.*  
*Pranas Budininkas*

Br  
Prangley, Baird, Clayton,  
Miller & Vogel,

Attys.

Feb. 12, 1963

P. BUDININKAS

3,077,285

TIN-NICKEL-PHOSPHORUS ALLOY COATINGS

Filed Sept. 15, 1961

6 Sheets-Sheet 5

FIG. 12



FIG. 13 Standard Specimen



FIG. 14A

INVENTOR.

Pranas Budininkas

BY

Prangley, Baird, Clayton,  
Meller & Vogel, / Atty's.

Feb. 12, 1963

P. BUDININKAS

3,077,285

TIN-NICKEL-PHOSPHORUS ALLOY COATINGS

Filed Sept. 15, 1961

6 Sheets-Sheet 6



FIG. 14B



FIG. 14C



FIG. 15

INVENTOR.

Pranas Budininkas

BY  
Prangley, Baird, Clayton,  
Mellen & Vogel,  
Attnys.

# United States Patent Office

3,077,285

Patented Feb. 12, 1963

1

3,077,285

TIN-NICKEL-PHOSPHORUS ALLOY COATINGS  
Pranas Budininkas, Gary, Ind., assignor to General  
American Transportation Corporation, Chicago, Ill., a  
corporation of New York

Filed Sept. 15, 1961, Ser. No. 138,443  
20 Claims. (Cl. 220—64)

The present invention relates to tin-nickel-phosphorus alloy coatings, and more particularly to articles of manufacture carrying such coatings. This application comprises a continuation-in-part of the copending application of Pranas Budininkas, Serial No. 95,262, filed March 13, 1961.

Heretofore, articles have been provided with nickel-phosphorus coatings upon the surfaces thereof by chemical deposition from a plating bath of the nickel cation-hypophosphite anion type and such coatings have been particularly advantageous because they can be applied to articles having a variety of compositions, sizes, shapes and configurations. Although such nickel-phosphorus coatings afford good protection in a variety of uses and a degree of protection at least equal to that of electrolytically deposited nickel, efforts have been made to improve the protective properties thereof because of the great convenience in producing such nickel-phosphorus coatings on a wide variety of base elements having substantially any desired shape. For example, various physical treatments of the nickel-phosphorus coatings have been developed to improve the protective properties thereof, such as the heat treatment disclosed in U.S. Patent No. 2,908,419, granted on October 13, 1959, to Paul Talmey and William J. Crehan.

Thus, it is a general object of the invention to provide an improved protective coating for an article of manufacture, and particularly an improved tin-nickel-phosphorus coating, wherein a nickel-phosphorus coating is first produced by chemical deposition from a plating bath of the nickel cation-hypophosphite anion type and then modified by diffusion tin plating.

Another object of the invention is to provide an improved article of manufacture comprising a body carrying an improved protective coating of nickel-phosphorus alloy intimately bonded thereto, the outer skin of the coating having tin diffused therein.

Yet another object of the invention is to provide as an article of manufacture, a body having a heat-hardened protective coating intimately bonded thereto and comprising a nickel-phosphorus alloy carrying substantial tin thermally diffused in the outer skin portion thereof.

Still another object of the invention is to provide an article of manufacture including a body having an improved protective coating thereon comprising a tin-nickel-phosphorus alloy.

Yet another object of the invention is to provide on an article of manufacture an improved protective coating of tin-nickel-phosphorus alloy which shows corrosion resistance toward basic solutions, neutral solutions and acidic solutions superior to that of electrolytically deposited nickel, nickel-phosphorus coatings, and electrolytically formed codeposits of tin and nickel.

Still another object of the invention is to provide an improved protective coating including a nickel-phosphorus alloy having a vapor deposited tin coating thereon.

A further object of the invention is to provide as an article of manufacture, a bearing member provided with a bearing surface comprising a nickel-phosphorus alloy having tin diffused therein.

Another object of the invention is to provide a bearing member provided with a bearing surface comprising a tin-nickel-phosphorus alloy.

2

A still further object of the invention is to provide a bearing member comprising a base metal support carrying a liner formed essentially of a nickel-phosphorus alloy, wherein the liner is provided with a bearing surface having tin diffused therein.

A further object of the invention is to provide on a workpiece an improved coating protecting the same against frictional wear, wherein the coating essentially comprises a tin-nickel-phosphorus alloy.

Further features of the invention pertain to the particular arrangement of the elements of the protective coatings on the articles or workpieces, whereby the above-outlined and additional operating features thereof are attained.

The invention, both as to its organization and method of operation, together with further objects and advantages thereof, will best be understood by reference to the following specification, taken in connection with the accompanying drawings, in which:

FIGURE 1 is a view in section through a typical article that can be coated in accordance with the present invention, the article being illustrated as comprising a base metal such as iron or the like;

FIG. 2 is a view in cross section, similar to FIG. 1, and showing a chemical nickel plating upon the upper surface of the base metal;

FIG. 3 is a view, similar to FIG. 2, showing a diffusion tin plating outer skin portion on the chemical nickel plating and being of the character and made in accordance with the principles of the present invention.

FIG. 4 is a view, similar to FIG. 3, but on a large scale and illustrating the coating obtained by one preferred embodiment of the present invention, the outer skin portion of the coating having separated into three discrete layers;

FIG. 5 is a view partly diagrammatic and partly in cross section of an apparatus suitable for carrying out the present process to produce an article having a protective coating in accordance with the principles of the present invention;

FIG. 6 is a graph showing the relation between the time of deposition of tin diffusion coatings on nickel-phosphorus coatings and the calculated thickness of the tin diffusion coatings, this relationship being illustrated for three separate combinations of the process variables;

FIG. 7 is a graph showing the relationship between the calculated thickness of tin diffusion coatings on nickel-phosphorus coatings and the ratio of nitrogen to hydrogen by volume in the reducing gas;

FIG. 8 is a view partly in cross-section and partly schematic illustrating the manner in which the principles of the present process can be applied to a hollow article made from several separate pieces whereby to produce a protective coating in accordance with the present invention;

FIG. 9 is a side elevational view of a railway tank car provided with a tank body incorporating a liner and embodying the present invention;

FIG. 10 is a greatly enlarged fragmentary view of a portion of a wall of the tank body of the railway car, taken in the direction of the arrows along the line 10—10 in FIG. 9;

FIG. 11 is a greatly enlarged fragmentary sectional view of another portion of the wall of the tank body of the railway car, taken in the direction of the arrows along the line 11—11 in FIG. 9;

FIG. 12 is a vertical sectional view of a bearing member provided with a liner and embodying the present invention;

FIG. 13 is a schematic end elevational view of a portion of an Amsler wear testing machine that is employed in testing the wearing qualities of materials and that was

utilized in certain tests of articles embodying the present invention; and

FIGS. 14A, 14B, 14C and 15 are graphic illustrations of test data obtained from the Amsler wear testing machine and involving test articles embodying the present invention.

Referring now to FIG. 1 of the drawings, there is illustrated diagrammatically an article generally designated by the numeral 10 which may be made of a base metal such as iron, or the like. In accordance with the present invention, a nickel-phosphorus protective coating is formed on the article 10, and after heat treatment, there is produced the article 20 illustrated in FIG. 2, in which a chemical nickel plating layer 22 containing, for example, about 92% nickel and 8% phosphorus by weight is shown on the exposed surface of the base metal 10 and intimately bonded thereto by means of an interface alloy layer 21 comprising essentially iron and nickel and phosphorus. In accordance with the present invention, the outer skin of the chemical nickel plating layer 22 can have tin applied thereto and diffused thereinto to produce a new article 30 of FIG. 3 having an alloy layer 31 on the outer surface thereof, the alloy layer 31 being a tin-nickel-phosphorus alloy having a variable content of tin therethrough with the tin being more highly concentrated adjacent to the outer surface thereof and gradually decreasing in concentration toward the layer 22. For example, the alloy layer 31 may have an average composition of approximately 45% tin, 51% nickel and 4% phosphorus by weight, thereby to provide the new article 30 having corrosion resistance properties superior to that of the article 20 illustrated in FIG. 2. As will be described more fully hereinafter, under certain operating conditions and in accordance with one preferred embodiment of the present invention, the diffusion tin plating outer skin portion 31 of FIG. 3 can be transformed so that it in fact contains three separate and distinct layers which are diagrammatically illustrated in FIG. 4 in the article 40. More specifically, the article 40 comprises, for example, a base metal 10 on which is superimposed the interface alloy layer 21 which is approximately 0.2 mil thick and comprises essentially iron and nickel and phosphorus. Upon the alloy layer 21 is the chemical nickel plating alloy layer which may have a thickness in the order of 1.4 mils and has a typical composition of 92% nickel and 8% phosphorus by weight. Disposed upon the alloy layer 22 is the layer 31 which in fact includes three separate layers, namely, an outer layer 41 approximately 0.25 mil thick high tin alloy, an intermediate layer 42 approximately 0.15 mil thick and comprising the nickel-phosphorus chemical nickel plating alloy distributed in tin, and a lower layer 43 approximately 0.3 mil thick and comprising tin distributed in the nickel-phosphorus nickel chemical plating alloy, the three layers 41, 42 and 43 corresponding to three different phases of the tin-nickel-phosphorus system.

It has now been found that the protective layers of the article 30 in FIG. 3 and the objects and advantages set forth above can be obtained by first producing a nickel-phosphorus chemical nickel plating coating upon the surface of the base material 10 by chemical deposition from a plating bath of the nickel cation-hypophosphite anion type and then converting to a tin-nickel-phosphorus alloy the outer skin of the coating by simultaneously depositing metallic tin upon the outer surface of the coating and by diffusing and alloying the tin into the outer skin of the coating. The tin is preferably deposited upon the nickel-phosphorus alloy by heating the coating to a temperature above the melting point of tin and below the melting point of the nickel-phosphorus coating and reducing to metallic tin a compound of tin upon the outer surface of the heated coating. The compounds of tin useful in the present invention are the tin halides, either stannous or stannic compounds being useful for this purpose, the preferred compound being stannous chloride. The tin

compound is preferably reduced by means of a reducing gas which contains hydrogen and can be produced by mixing nitrogen and hydrogen, by cracking ammonia or by thermally cracking natural gas. It has been found that coatings having improved appearances are obtained if sufficient hydrogen is present in the reducing gas, gray coatings of tin being obtained if the ratio of nitrogen to hydrogen by volume is above 3.5 and more desirable semi-bright tin deposits being obtained if the ratio of nitrogen to hydrogen by volume is less than 3.5, a preferred concentration of the hydrogen in the reducing gas being in the range of 25% to about 40% by volume. The reaction is carried out at a temperature preferably above the melting point of tin, i.e., 332° C., and below the melting point of the nickel-phosphorus alloy, i.e., 880° C., the preferred range of temperature being from about 400° C. to about 630° C., the optimum operating temperature being 630° C. In carrying out the process the tin compound is volatilized and mixed with the reducing gas and the resultant mixture applied to the heated nickel-phosphorus surface, the various reaction variables being selected so that the rate of deposition of metallic tin upon the nickel-phosphorus surface is less than the rate of diffusion of metallic tin into the nickel-phosphorus coating. It also has been found that it is desirable to have a substantial nickel-phosphorus coating to give good corrosion protection and preferably the coating should be at least about 2 mils thick and may be even thicker to give optimum corrosion resistance for the tin-nickel-phosphorus alloy coating formed.

The nickel-phosphorus layer 22 may be produced from any of the well-known nickel cation-hypophosphite anion plating baths. More particularly, the chemical plating bath employed may be any one of a number of available compositions, such, for example, as disclosed in U.S. Patent No. 2,532,283 granted on December 5, 1950, to Abner Brenner and Grace E. Riddell; U.S. Patent No. 2,658,841 granted on November 10, 1953, to Gregoire Gutzeit and Abraham Krieg; or U.S. Patent No. 2,658,842 granted on November 10, 1953, to Gregoire Gutzeit and Ernest J. Ramirez. However, it is preferable that this chemical plating bath be of the composition of that disclosed in U.S. Patent No. 2,822,294 granted on February 4, 1958, to Gregoire Gutzeit, Paul Talmey and Warren G. Lee, since this particular plating bath is admirably suited to a continuous plating process. The chemical plating bath of the Gutzeit, Talmey and Lee patent mentioned essentially comprises an aqueous solution of a nickel salt, a hypophosphite, a complexing agent selected from the group consisting of lactic acid and salts thereof, and an exalting additive selected from the group consisting of propionic acid and salts thereof. In this plating bath, the absolute concentration of hypophosphite ions is within the range 0.15 to 1.20 moles per liter, the ratio between the concentrations of nickel ions and hypophosphite ions is within the range 0.25 to 1.60, the absolute concentration of lactic ions is within the range 0.25 to 0.60 mole per liter, the absolute concentration of propionic ions is within the range 0.025 to 0.060 mole per liter, and the pH is within the approximate range 4.0 to 5.6.

In the chemical plating of the upper exposed surface of the base metal 10, the plating bath is continuously circulated across the exposed surface and through the associated continuous plating system, not shown, with regeneration of the plating bath, as time proceeds, in order to maintain substantially the composition thereof set forth, as is disclosed in U.S. Patent No. 2,717,218, granted on September 6, 1955, to Paul Talmey and William J. Crehan. In this method, the temperature of the plating bath contacting the base metal 10 is maintained near the boiling point thereof, at about 210° F., so as to obtain a high plating rate in the production of the coating 22; and the plating step is continued throughout an appropriate time interval in order to obtain the desired thickness of

the coating 22, the plating rate of the plating bath mentioned being about 1 mil per hour. Normally the thickness of the coating 22 is at least about  $\frac{1}{2}$  mil and usually in the approximate range 1 to 5 mils, a thickness of about 1.5 to 2.0 mils being recommended for general utility.

The coating 22, as chemically deposited, is in the form of a layer intimately bonded to the surface of the base metal 10 and comprises an amorphous solid material consisting essentially of a metastable undercooled solution of phosphorus in nickel, and including about 88 to 94% nickel, and 6 to 12% phosphorus by weight, the coating 22 being characterized by adhesion, wear resistance, and resistance to corrosive attack by ordinary acids, bases, and other reagents, comparable to electro-deposited nickel. As chemically deposited, the coating 22 has a hardness corresponding to a Vickers hardness number (V.H.N.) of about 525. The variable composition of the coating 22 with respect to the inclusion of nickel and phosphorus is dependent on pH and, to a limited extent, upon the concentration of the hypophosphite in the plating bath, and also upon the concentration of phosphite in the plating bath, it being understood that as the plating reactions proceed at the catalytic surfaces of the base metal 10, the hypophosphite ions are oxidized to phosphite anions as the nickel cations are correspondingly reduced to metallic nickel and deposited upon the catalytic surface of the metal comprising the workpiece 10. With certain types of chemical nickel plating baths and utilizing certain systems of deposition, it is possible to obtain a coating 22 having nickel and phosphorus content outside of the ranges specified above and more particularly it is possible to obtain coatings including from about 85% to 97% nickel and from about 3% to 15% phosphorus by weight.

As noted above, the chemical deposition of the coating 22 upon the workpiece 10 involves the catalytic plating reactions mentioned, whereby the workpiece 10 must be formed of catalytic material or must have growth nuclei of catalytic material thereon. While there are a great number of catalytic materials upon which the chemical deposition may take place, the ordinary catalytic materials conventionally comprise iron and its alloys, copper and its alloys, and aluminum and its alloys. For example, the material of the workpiece might be: iron, carbon steel, chrome steel, cobalt steel, silicon steel, manganese steel, nickel steel, molybdenum steel, nickel-cobalt steel, nickel-chrome steel, chrome-manganese steel, manganese-molybdenum steel, chrome-copper-nickel steel, copper, brass, bronze, silicon bronze, Phosphor bronze, beryllium-copper, cadmium-copper, chromium-copper, nickel-copper, aluminum, aluminum-brass and aluminum-bronze. If the workpiece 10 is not formed of one of the above materials, it may be desirable to affix to the exposed surface thereof growth centers of catalytic metal, the growth centers being applied, for example, by means of the process set forth in U.S. Patent No. 2,690,401, granted on September 28, 1954, to Gregoire Gutzeit, William J. Crehan and Abraham Krieg, and U. S. Patent No. 2,690,402, granted on September 28, 1954, to William J. Crehan. On the other hand, if the workpiece 10 is formed of certain metals such as magnesium or titanium, it must be treated in a particular manner to obtain a satisfactory coating thereon, the method of treating titanium, zirconium and hafnium being set forth in U.S. Patent No. 2,928,757, granted on March 15, 1960, to Warren G. Lee and Emilian Browar, and the method of treating articles made of magnesium and its alloys being set forth in U.S. Patent No. 2,983,634, granted on May 9, 1961, to Pranas Budininkas.

In accordance with the present process the workpiece 10 with the protective coating 22 of nickel-phosphorus thereon can be treated to increase the corrosion resistance of the coating 22 by forming a diffusion coating 31 of tin on the outer skin portion thereof. The diffusion tin coating process can conveniently be carried out in the appa-

ratus 500 illustrated in FIG. 5 of the drawings. In the system 500 ammonia gas may be used as a source of hydrogen that serves as the reducing agent and a halide of tin may be used as the source of tin. The ammonia gas is fed from a line 501 to a flow meter 502 from which the measured stream of ammonia gas flows through a line 503 to an inlet of a ceramic tube 504 disposed within a furnace 505 and containing therein a mass 506 of steel wool; the steel wool when heated to about 930° C. catalyzes the cracking of ammonia gas to produce free nitrogen and free hydrogen. The mixture of nitrogen and hydrogen together with any other uncracked ammonia is fed by a line 507 to a first manually operable valve 508 and a second manually operable valve 519. The other side of the valve 508 connects with a line 509 which is connected to a container or chamber 510 for the tin halide through an inlet connection 511 therefor. In order to heat the tin halide within the container 510 to the necessary vaporizing temperature, a suitable heater 512 which may be electrically operated surrounds the container 510. An outlet connection 513 is provided for the container 510 and is adapted to receive therethrough the stream of reducing gas that enters at the inlet 523, the stream of reducing gas sweeping across the surface of the tin halide in the container 510 to entrain and mix therein quantities of the vaporized tin halide. The outlet connection 513 is one leg of a Y-connection, another leg of the Y-connection being an elongated tube 514 extending through a heat exchanger 520 and into substantially the center of a reaction chamber 531. The heat exchanger 520 is of the counter-current type and includes a cylindrical housing 521 enclosing a substantial portion of the tube 514, a gas inlet 523 disposed within the container 531 and an exhaust 524 at the other end of the housing 521. Exhaust gases from the reaction chamber 531 can flow through the inlet connection 523, through the space 522 between the tube 514 and the housing 521 and out through the exhaust 524, the outgoing gases giving up a substantial portion of the sensible heat therein to the incoming reaction gases to aid in raising the temperature of the reaction gases to that within the reaction chamber 531. The reaction chamber 531 is disposed within a furnace 530 capable of maintaining the reaction chamber 531 and the contents thereof at the desired reaction temperature and may be, for example, a "Waltz" furnace which is an automatic resistance type electric furnace. Means is provided to suspend one or more of the workpieces 20 therein and a thermocouple well 534 is also provided to receive therein a thermocouple 535 connected to the controller for the furnace 530.

#### EXAMPLE 1

Utilizing the system 500 of FIGURE 5, nickel-phosphorus coatings were converted to tin-nickel-phosphorus coatings on mild steel specimens rectangular in shape and having approximately 20 sq. cm. of surface area. First a nickel-phosphorus coating was applied to the steel specimens utilizing the method disclosed above and explained in greater detail in U.S. Patent No. 2,822,294 to provide thereon a nickel-phosphorus coating having a thickness of approximately 2 mils. A quantity of anhydrous stannous chloride was placed in the container 510 and the heater 512 placed in operation. The valve 508 was closed and a bypass valve 519 opened, the valve 519 interconnecting the line 507 with the reaction gas tube 514 via a line 516 and the third leg 515 of the Y-connection. The furnace 505 is then placed in operation and heated to about 930° C. after which ammonia gas is introduced into the tube 504 where about 99% of the ammonia gas is cracked to form a mixture of hydrogen and ammonia containing about 75% of hydrogen by volume. The gases are fed through the line 507 to the valve 519 to the line 516 to the inlet 515 and the conduit 514 into the reaction chamber 531 in order to purge the air from the reaction chamber 531 while the furnace 530 is being

heated. After about 30 minutes of purging by means of the reducing gas, all of the furnaces are at the operating temperature, the furnace 505 being operated at approximately 530° C. and the furnace 512 at about 480° C. and the furnace 530 at about 630° C. The valve 508 is then opened and the valve 519 closed whereby the reducing gas is now conveyed by means of the line 509 to the input connection 511 of the chamber 510 whereby the reducing gas is mixed with the stannous chloride vapors within the chamber 510, the mixture being conveyed through the outlet conduit 513 and the tube 514 to the interior of the reaction chamber 531. The mixture of the stannous chloride and the reducing gas impinges upon the surface of the workpiece 20 whereupon a portion of the stannous chloride is reduced to metallic tin, the metallic tin being well above its melting point of 332° C. The molten tin proceeds to alloy with and diffuse into the nickel-phosphorus coating 22 upon the workpiece 20. The reaction gases then pass into the inlet connection 523 to the heat exchanger 520 and through the passage 522 therein and out through the exhaust 524, the exhaust gases serving to heat the incoming reaction gases whereby to conserve energy within the system. Preferably, the exhaust 524 is held under a pressure equal to approximately 2 inches of water so that the pressure within the reaction chamber 531 is slightly higher than atmospheric pressure. The reaction is continued for a suitable period of time and in a typical example the reaction proceeded for two hours. The workpiece 20 was then removed and was found to have gained 0.0721 gram in weight and it was found that the resultant diffusion tin plating had a thickness of 0.197 mil. The diffusion tin coating 31 was semi-bright and gray in color, was evenly applied and thoroughly covered the workpiece 20.

It was found that when the coating 31 was applied to a nickel-phosphorus coating 22 containing 92% nickel and 8% phosphorus by weight, the composition of the layer 31 was within the following ranges: from about 40% to about 50% tin, from about 46% to about 56% nickel, and from about 4% to about 5% phosphorus by weight. However, the composition of the coating 22 may vary substantially as has been explained above and may contain from about 85% to about 97% nickel and from about 3% to about 15% phosphorus by weight, and accordingly, the layer 31 may have a composition which varies substantially and may contain from about 1% to about 50% tin and from about 46% to about 93% nickel and from about 3% to about 12% phosphorus by weight.

It has been found that there are several competing reactions which may be taking place within the reaction chamber 531 as follows:

(1) Catalytic reduction (when hydrogen is present).



(2) Autoreduction-oxidation.



(3) Replacement of nickel with tin.



When hydrogen is present, reaction No. 1 above predominates and there is substantially no tin deposited by means of the mechanisms of reactions No. 2 and No. 3. In the absence of hydrogen, the reaction No. 2 tends to dominate, deposition proceeding by the autoreduction-oxidation process. In no event is reaction No. 3 of any substantial significance. None of the reactions have any substantial conversion at equilibrium but reasonable deposition rates are obtained under non-equilibrium condi-

tions where reactants are provided in a surplus and the reaction products are continuously removed. The nickel-phosphorus coating 22 has also been found to be a catalyst for the reduction of tin in accordance with reaction No. 1 above and is a substantially better catalyst than other metals including tin.

The diffusion tin coating 31 is substantially superior to the nickel-phosphorus coating 22 as regards corrosion resistance to common chemicals and there is set forth in Table 1 a comparison of the corrosion resistance of the workpiece 30 with the corrosion resistance of the workpiece 20, the workpiece 30 having as the outer skin portion thereof a tin-nickel-phosphorus alloy and the workpiece 20 having as the outer skin portion thereof a nickel-phosphorus coating as plated, the figures given being the corrosion rate in mils per year.

Table 1

[Corrosion rate, mils per year]

| Commodity                                                                    | Nickel-Phosphorus Coating | Tin-Nickel-Phosphorus Coating |
|------------------------------------------------------------------------------|---------------------------|-------------------------------|
| Ammoniated Ammonium Nitrate, 30% ammonia and 40% ammonium nitrate, by Weight | 2.20                      | 0.180                         |
| Ammonium Hydroxide, 28-30% ammonia, by Weight                                | 0.98                      | 0.020                         |
| Ammonium Nitrate 30%, by Weight                                              | 8.24                      | 0.053                         |
| Citric Acid, 5% by Weight                                                    | 2.66                      | 0.610                         |
| Dry Sherry Wine                                                              | 0.94                      | 0.000                         |
| Ferric Sulfate, 1% by Weight                                                 | 25.80                     | 0.520                         |
| Lactic Acid, 50% by Weight                                                   | 0.93                      | 0.179                         |
| Lactic Acid, 80% by Weight                                                   | 0.37                      | 0.006                         |
| Sauterne Wine                                                                | 1.36                      | 0.980                         |
| Sulfuric Acid, 10% by Volume                                                 | 16.20                     | 3.450                         |

The above corrosion rates were obtained by test procedure which included immersing the test specimens in the various solutions at 30° C. with complete immersion and no aeration. All the test specimens used had 20 sq. cm. of surface area and were immersed in 100 ml. of solution either by suspending the specimen from a glass hook or by resting the two lower corners thereof on the bottom of a test tube. Tests with very volatile liquids were performed in sealed tubes; tests with less volatile solutions were performed with the tubes closed with rubber stoppers equipped with condenser tubes; and tests with non-volatile solutions were performed in open test tubes. All dilute solutions were changed once a week. The weight loss and the appearance of the solutions were checked periodically, and at least once a week. If no earlier failure was observed, the tests were continued for a total of three to six weeks. Whenever penetration through the nickel-phosphorus coating or the tin-nickel-phosphorus coating was observed, the test was discontinued and the corrosion rate was calculated in mils per year using the weight loss from the time of termination of each test; however, for specimens failing before the termination of the tests, the corrosion rate was calculated using the time at the inspection prior to the failure. The density of the tin-nickel-phosphorus alloy lies between the density of tin and the density for the nickel-phosphorus coating which is heavier than tin but for the purpose of determining the corrosion rates, the density of tin was used in the calculations, thereby to obtain conservative estimates of the corrosion rates, i.e., the corrosion rates obtained in this manner are slightly higher than if they would be using the actual density of the tin-nickel-phosphorus alloy.

The corrosion tests results consistently indicated that the tin-nickel-phosphorus alloy possessed corrosion resistance superior to the nickel-phosphorus coating in the following solutions: ammonium hydroxide, 28-30% ammonia by weight; ammoniated ammonium nitrate, 30% ammonia and 40% ammonium nitrate by weight; ammonium nitrate, 30% by weight; acetaldehyde; formaldehyde; acetic anhydride; glacial acetic acid; acetic acid, 5% by weight; lactic acid, 50% and 80% by weight; citric acid, 5% by weight; ferric sulfate, 1% by weight; sulfuric acid,

10% by volume; nitric acid, concentrated (70% HNO<sub>3</sub> by weight), and 20% by volume; dry sherry wine; and sauterne wine. The tin-nickel-phosphorus alloy provides sufficient protection in ammoniacal and weakly basic solutions that it can be used in commercial applications where the nickel-phosphorus alloy has not been used heretofore because of the relatively high corrosion rate thereof. In general, the tin diffusion coating 31 shows good corrosion resistance toward basic solutions, neutral solutions, and acidic solutions, the tin-nickel-phosphorus alloy thereof being readily soluble only in aqua regia.

The tin-nickel-phosphorus alloy in the coating 31 differs in other physical properties from the nickel-phosphorus alloy in the coating 22 and from the coatings of tin and nickel electroplated in a manner such that the tin and nickel are laid down simultaneously to form a single homogeneous coating. For example, the tin-nickel-phosphorus alloy of the coating 31 is a solid at temperatures well above the melting point of tin. The tin-nickel-phosphorus alloy in a typical specimen has a hardness corresponding to a point within the range V.H.N. 750 to 950; whereas the electro-plated tin-nickel coating has a hardness corresponding to about V.H.N. 700.

It is essential in producing a satisfactory tin diffusion coating 31 that the metallic tin be deposited upon the surface of the nickel-phosphorus coating at a rate less than the diffusion rate of tin into the nickel-phosphorus coating. If the metallic tin is in fact deposited at a rate greater than the diffusion rate of tin into the nickel phosphorus coating, the excess tin either covers the surface in a manner to prevent further catalytic reduction of tin thereon or balls up and rolls from the surface whereby to remove the metallic tin from contact with the nickel-phosphorus coating. In this regard it is noted again that although the nickel-phosphorus coating is a good catalyst for the reduction of stannous chloride by hydrogen, tin itself is not a good catalyst and the reaction will not take place upon a surface of tin. In fact, a convenient way of treating the various parts of the reaction chamber 510, the heat exchanger 520 and reaction chamber 531 to minimize loss of tin by spurious reduction thereof is to coat these parts with the tin-nickel-phosphorus alloy. This can be conveniently done by first applying a nickel-phosphorus coating as explained above and then carrying out the reaction of the present process therein whereby to form upon the nickel-phosphorus coating a tin-nickel-phosphorus alloy.

The rate of deposition of tin upon the surface of the article being coated increases with an increase in the temperature within the reaction chamber 531. In order to determine the relationship between the reaction temperature and the amount of tin deposited upon the workpiece, workpieces were utilized having three square inches of surface area and were coated in the reaction chamber 531 using cracked ammonia gas as the reducing agent, the ammonia being 99% cracked and being supplied at the rate of 1600 cc. per minute. The temperature of the stannous chloride was maintained at 480° C. and the coating was carried out for a period of three hours. At the end of three hours the specimens were removed from the reaction chamber 531 and weighed to determine the increase in weight thereof. The following is a summary of the weight gains ascertained for a plurality of reaction temperatures in Examples 2 to 6:

The rate of diffusion of atomic tin into the nickel-phosphorus alloy also increases as the temperature of the workpiece increases and for this additional reason the preferred operating temperature is the higher temperature of 630° C. Even higher rates of deposition of atomic tin

5 can be obtained at temperatures above about 630° C., but it has been found that in general the base metal 10 should not be heated above this temperature and the rate of diffusion does not increase with temperature as rapidly as does the rate of deposition of tin, and as a result metallic tin would be deposited at a rate greater than that at which it can be diffused into the nickel-phosphorus alloy and, accordingly, the additional tin would be lost from the coating operation, the excess tin balling up and rolling 10 off of all inclined surfaces and coating and stopping the reaction on surfaces from which the balled up tin cannot drain.

15 The rate of decomposition of the metallic tin is also a function of the partial pressure of hydrogen in the gases flowing into the reaction chamber 531 and the partial pressure of the tin compound in those gases as well as the reaction temperature in the reaction chamber 531. The effect of the partial pressure of hydrogen in the reducing gas is best illustrated in FIG. 7 of the drawings wherein

20 there is summarized the results of a group of examples of coating operations carried out in the system 500 of FIGURE 5. Each of the examples plotted in FIGURE 7 was carried out at a reaction temperature of 630° C. and the partial pressure of the stannous chloride in the reaction gasses was maintained constant by heating the stannous chloride to a temperature of 480° C. The coating reactions were carried out for a time period of two hours on specimens having a surface area of 80 sq. cm. The weight

25 gain of the specimens was determined and a thickness of the tin-nickel-phosphorus alloy coating calculated and plotted on the vertical axis of FIGURE 7. The partial pressure of the hydrogen gas in the reducing gas was expressed as the ratio by volume of nitrogen to hydrogen and plotted on the horizontal axis in FIGURE 7. In order accurately to control the ratio of nitrogen to hydrogen in the reaction gases, a mixture of hydrogen and nitrogen gases was used in the place of cracked ammonia gas. To this end the system 500 in FIGURE 5 is provided with a connection 541 to a source of hydrogen (not shown), the connection 541 communicating with a flow meter 542 which in turn is connected through a line 543 to a furnace 545 in which the hydrogen gas is heated. The outlet from the furnace 545 is connected through a line 547 to two manually operable control valves 548 and 549, the outlet of the control valve 548 being connected to the line 509 and the outlet of the control valve 549 being connected to the line 516, whereby all or a portion of the heated hydrogen gas can be passed through the

30 chamber 510 to pick up stannous chloride vapors for inclusion in the reaction gases. A connection 551 is provided and adapted to be connected to a source of nitrogen gas (not shown), the connection 551 communicating with a flow meter 552 having the output thereof connected to a furnace 555 through a line 553. The furnace 555 is adapted to heat the incoming nitrogen gas and the output of the furnace 555 is connected to a line 557 which in turn connects to two manually operable control valves 558 and 559, the control valve 558 connecting to the line 509 and the control valve 559 connecting to the line 516.

35 Any desired portion of the heated stream of nitrogen gas can be passed through the chamber 510 to sweep stannous chloride vapors therewith into the reaction chamber 531.

40 Three rates of total gas flow were also utilized to obtain the data plotted in FIG. 7, the data indicated by a circle being obtained using a total gas flow of 60 cc. per minute, the data designated by a triangle being obtained using a total gas flow of 100 cc. per minute and the data designated by a square being obtained by a gas flow of

45 150 cc. per minute. The following table lists the thick-

| Example No. | Reaction Temperature, °C. | Weight Gain, milligrams |
|-------------|---------------------------|-------------------------|
| 2           | 510                       | 43.4                    |
| 3           | 525                       | 47.0                    |
| 4           | 592                       | 60.0                    |
| 5           | 610                       | 78.7                    |
| 6           | 630                       | 86.4                    |

50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930

## 11

ness of the tin-nickel-phosphorus alloy coating calculated for each of the three rates of total gas flow for various ratios of nitrogen gas to hydrogen gas by volume:

Table 2

| Ratio of Nitrogen to Hydrogen<br>By Volume | Thickness of Tin-Nickel-Phosphorus Coating in Mils |              |              |
|--------------------------------------------|----------------------------------------------------|--------------|--------------|
|                                            | 60 cc./min.                                        | 100 cc./min. | 150 cc./min. |
| 0.....                                     | 0.280                                              | 0.225        | 0.230        |
| 1.....                                     | 0.218                                              | 0.210        | 0.213        |
| 2.....                                     | 0.203                                              | 0.199        | .....        |
| 3.....                                     | .....                                              | 0.172        | 0.192        |
| 4.....                                     | .....                                              | .....        | .....        |
| 5.....                                     | 0.175                                              | .....        | .....        |
| 8.....                                     | .....                                              | .....        | 0.171        |
| 11.....                                    | 0.165                                              | .....        | .....        |
| 19.....                                    | 0.160                                              | .....        | .....        |

The thickest deposit of tin-nickel-phosphorus alloy coating was obtained when the reducing gas comprised only hydrogen (the nitrogen to hydrogen ratio being 0), a coating of 0.2 mil having been obtained at a gas flow of only 60 cc./min. This coating was gray in color and semi-bright in luster as were all coatings obtained with a nitrogen to hydrogen ratio by volume less than about 3.5. When using nitrogen to hydrogen ratios by volume greater than about 3.5, the deposits obtained were dull in luster and gray in color and had a generally less desirable appearance than those coatings obtained with nitrogen to hydrogen ratios less than about 3.5. It is noted that the thickness of the coatings did not decrease substantially with further dilution of the hydrogen gas after a ratio of approximately 5 and it is believed that the auto-reduction-oxidation reaction becomes a significant if not the dominant reaction taking place when the partial pressure of the hydrogen gas becomes so small. Accordingly, it is preferred that the partial pressure of hydrogen in the reaction gases correspond to a nitrogen to a hydrogen ratio by volume of less than about 3.5 and that the hydrogen constitutes approximately 25% by volume of the reducing gas and up to about 40% by volume, the preferred amount being about 33% by volume of the reducing gas.

Other reducing gases can be used in the place of cracked ammonia and the nitrogen-hydrogen mixtures discussed above. For example, anhydrous ammonia may be used as the reducing gas without prior cracking thereof, the ammonia gas being heated, mixed with the stannous chloride and the mixture applied against the surface of the workpiece in the reaction chamber 531. When the gas strikes the nickel-phosphorus coating, part of the ammonia is disassociated producing hydrogen which reduces the stannous chloride vapor to metallic tin. The deposited tin then diffuses into the nickel-phosphorus coating forming the nickel-tin alloy described above. The hydrogen chloride which is produced as a result of the reaction reacts with the excess ammonia present forming ammonium chloride which is removed from the reaction zone by the sweep of the reaction gases. The total reaction can be expressed as follows:



Thus theoretically  $2\frac{2}{3}$  moles of ammonia are required to deposit one mole of tin. The following is a preferred example utilizing heated anhydrous ammonia as the reducing gas.

## EXAMPLE 7

The reaction chamber 531 is heated to a temperature of  $630^{\circ}\text{C}$ . and purged of air by means of ammonia gas for one-half hour. The stannous chloride is heated to a temperature of  $480^{\circ}\text{C}$ . Four test specimens or metal coupons having a surface area of 20 sq. cm. each are

## 12

disposed within the reaction chamber 531. After purging the reaction chamber 531, the ammonia was swept across the heated stannous chloride at a rate of 60 cc./min. and the reaction continued for four hours. Each coupon had a weight gain of 0.0963 gram corresponding to a calculated thickness of the tin-nickel-phosphorus coating of 0.261 mil. The coating was gray in color and uniform throughout the surface of the coupon.

Cracked natural gas can also be used as the reducing gas in the present reaction. The following is an example of this reaction:

## EXAMPLE 8

Natural gas was thermally cracked using an air to gas ratio of two to one to produce a resultant gas containing about 30% hydrogen by volume. The cracked natural gases were utilized to coat a workpiece, the reaction being carried out at a temperature of  $630^{\circ}\text{C}$ . with the stannous chloride maintained at a temperature of  $555^{\circ}\text{C}$ . and using a gas flow of 55 cc./min. for four hours. A workpiece having a surface area of 20 sq. cm. had a weight gain of 0.0788 gram corresponding to a calculated thickness for the tin-nickel-phosphorus alloy of 0.21 mil. The resultant coating was gray in color and continuous throughout the surface area of the workpiece and was generally brighter than the coatings obtained using anhydrous ammonia as the reducing gas.

The stannous chloride utilized as the source of tin in all of the preceding Examples 1 through 8 has a boiling point of  $620^{\circ}\text{C}$ . and it is preferred to maintain the temperature of the stannous chloride in the chamber 510 well below the boiling point thereof in order to obtain the desired concentration of hydrogen at the surface of the workpiece where the tin reduction reaction is to be carried out and in general it has been found desirable to maintain the temperature of the stannous chloride in the range from about  $480^{\circ}\text{C}$ . to about  $500^{\circ}\text{C}$ ., the preferred temperature being about  $480^{\circ}\text{C}$ . When the stannous chloride is held at  $480^{\circ}\text{C}$ ., a sufficient amount of stannous chloride vapor is present at the nickel-phosphorus reaction surface with manageable flow rates for the reducing gas and the partial pressure of hydrogen in the reducing gas or the hydrogen formed by the association of ammonia on the nickel-phosphorus surface is sufficient to reduce the stannous chloride at a rate to deposit metallic tin at a rate less than the rate of diffusion of tin into the nickel-phosphorus coating. In fact the amount of stannous chloride present is more than sufficient to provide an excess at the reaction surface under the conditions of the reaction set forth in Examples 1 to 8. The use of higher temperatures for the stannous chloride simply results in the recycling of even more stannous chloride, assuming that the stannous chloride is cooled at the exhaust outlet 524 and purified for reuse in the reaction.

It is believed that the reduction of tin compounds by hydrogen is catalytic in nature, the nickel-phosphorus coatings acting as a good catalyst and the tin-nickel-phosphorus alloy not appreciably catalyzing the tin reduction reaction. Accordingly, as the reaction progresses the rate of deposition of metallic tin decreases as the available nickel-phosphorus coating surface is covered by the tin-nickel-phosphorus alloy. There is shown in FIG. 6 of the drawings the results of three series of experiments illustrating that the rate of deposition of metallic tin decreases with time, the rate of deposition being more rapid at the beginning of the reaction period and steadily declining as the reaction proceeds. There is plotted in curve 601 the results of a series of runs in which a nitrogen-hydrogen gas mixture was utilized as the reducing gas, the ratio by volume of nitrogen to hydrogen being two to one. The reactions were carried out at  $630^{\circ}\text{C}$ ., the stannous chloride being maintained at  $480^{\circ}\text{C}$ . and the reducing gas flow being 60 cc./min. It is clear from the curve 601 that the rate of deposition is maxi-

mum during the first part of the reaction period and then steadily decreases. Runs maintained for periods longer than 10 hours show substantially no further deposition of atomic tin upon the workpieces. On the curve 602 are plotted the calculated thicknesses in mils of the tin-nickel-phosphorus alloy coatings obtained using cracked natural gas as the reducing gas at a reaction temperature of 630° C., the stannous chloride being maintained at a temperature of 550° C. and the reducing gas flow being 55 cc./min. Again the rate of deposition of tin is higher at the beginning of the reaction and steadily declines. There are plotted on the curve 603 the results of utilizing anhydrous ammonia as the reducing gas at a reaction temperature of 510° C., the stannous chloride being maintained at 510° C. and the reducing gas flow being 25 cc./min. Here again the reaction rate is highest at the beginning of the reaction and steadily decreases with time.

In all cases, the tin-nickel-phosphorus alloy coating obtained at a reaction temperature of 630° C. during the reaction time of less than 4 hours shows substantially only a single layer as illustrated in FIG. 3 of the drawings, this being the layer 31 labeled "Diffusion Tin Plating Outer Skin Portion." In a typical example, this alloy layer will have an average composition of 45% tin, 51% nickel and 4% phosphorus, by weight, it being understood that the amount of tin may be greater or less depending upon the various reaction conditions. After the tin reduction reaction has been carried on for four hours or longer, the coating 31 forms into three separate layers illustrated in FIG. 4 of the drawings and designated by the numerals 41, 42 and 43. In this case the outermost layer 41 consists essentially of tin with relatively small amounts of the nickel-phosphorus alloy distributed therein. The second layer 42 comprises predominantly tin in which is distributed a small amount of nickel-phosphorus chemical nickel plating alloy. The third layer 43 comprises predominantly the nickel-phosphorus chemical nickel plating alloy in which is distributed a small amount of tin. It is believed that the original unitary coating 31 of diffusion tin in a nickel-phosphorus coating approaches equilibrium after being heated for about four hours and separates into the layers 41, 42 and 43 which represent the various possible combinations of ingredients for a system containing tin and nickel and phosphorus. In this regard it is noted that the tin definitely diffuses into the nickel-phosphorus coating inasmuch as tin is present at depths several times the thickness of the tin coating to be expected by calculation from the gain in weight. For example, in certain specimens in which the weight gain indicated a thickness of the tin layer of 0.49 mil, tin was present throughout a layer that was 1.05 mils thick.

The protective coating of FIG. 4, i.e., a coating in which the reaction has been carried out for a sufficient length of time to produce three distinct layers containing tin, shows substantially better corrosion resistance than do those tin-nickel-phosphorus protective coatings consisting of only one layer produced in the reaction carried out for less than four hours. Although the longer reaction time does deposit additional tin, the difference in corrosion rates indicates a change in character of the protection afforded in excess of that expected from the added tin deposited during the additional reaction time, particularly in view of the fact that the amount of tin deposited during the later portions of the reactions are substantially less than those deposited during the initial portion of the reaction. It is believed that the three layer tin-nickel-phosphorus alloy formation illustrated in FIG. 4 of the drawings serves further to cover any minute imperfections and thus greatly enhances the corrosion protection characteristics of the protective layer 31. Table 3 below summarizes the results of corrosion tests carried out on workpieces having thereon a nickel-phosphorus coating 2 mils thick to which is applied metallic

tin by the process of the present invention, the tin being applied for periods of two hours, four hours and six hours, respectively, on the various specimens. The corrosion tests were carried out in the same manner described above when discussing generally the corrosion resistance of the article 30. The figures given for the corrosion rate data are in mils of corrosion per year.

Table 3

| 10 | Commodity               | Tin Deposit, G./20 cm. <sup>2</sup>            | Corrosion Rate, Mils Per Year             |                                           |                                           |
|----|-------------------------|------------------------------------------------|-------------------------------------------|-------------------------------------------|-------------------------------------------|
|    |                         |                                                | 2 Hour Deposition                         | 4 Hour Deposition                         | 6 Hour Deposition                         |
| 15 | Lactic Acid, 80%-----   | 0.0753<br>0.0795<br>0.0780<br>0.1203<br>0.1310 | 0.036<br>0.020<br>0.038<br>-----<br>0.277 | -----<br>-----<br>-----<br>-----<br>0.101 | 0.008<br>0.006                            |
| 20 | Acetic Acid, 5%-----    | 0.0769<br>0.0756<br>0.1384<br>0.1338<br>0.1352 | 0.046<br>0.043<br>0.116<br>0.043<br>0.023 | -----<br>-----<br>-----<br>-----<br>0.412 | -----<br>-----<br>-----<br>-----<br>0.018 |
| 25 | Ferric Sulfate, 1%----- | 0.0736<br>0.0768<br>0.0789<br>0.1278<br>0.1303 | 0.116<br>0.116<br>0.412<br>-----<br>0.47  | -----<br>-----<br>-----<br>0.29           | 0.007<br>0.001                            |
| 30 |                         | 0.1337<br>0.1811<br>0.1785                     | 0.1337<br>0.1811<br>0.1785                | 0.29<br>-----<br>-----                    | -----<br>-----<br>-----                   |

It has also been found that it is preferred to deposit the metallic tin upon nickel-phosphorus coatings having a thickness of about at least 2 mils in order to permit formation of the three discrete layers 41, 42 and 43 illustrated in FIG. 4 and still provide a substantial layer 22 of a nickel-phosphorus coating in which no tin is present. Although tin-nickel-phosphorus alloy coatings produced upon nickel-phosphorus coatings that are less than 2 mils thick are entirely satisfactory for certain purposes, substantially increased corrosion resistance of the composite coating is realized if the nickel-phosphorus coating upon which the atomic tin is deposited has a thickness of at least 2 mils. There is set forth in Table 4 the results of corrosion tests conducted on specimens which have substantially the same amount of atomic tin deposited on nickel-phosphorus coatings having different thicknesses of 1 mil, 1.5 mils, and 2 mils, respectively. The corrosion rate data with respect to three common chemicals are given for illustrative purposes, the actual deposit of tin in grams for each 20 sq. cc. of specimen also being indicated. The corrosion rate data are in mils of corrosion per year.

Table 4

| 55 | Commodity                                                | Tin Deposit, G./20 cm. <sup>2</sup>            | Corrosion Rate, Mils Per Year           |                                          |                        |
|----|----------------------------------------------------------|------------------------------------------------|-----------------------------------------|------------------------------------------|------------------------|
|    |                                                          |                                                | 1 Mil                                   | 1.5 Mil                                  | 2 Mil                  |
| 55 | 1. Ammonium Nitrate, 30% by weight-----                  | 0.1184<br>0.1168<br>0.1177<br>0.1467<br>0.1320 | -----<br>-----<br>0.12<br>0.12<br>0.053 | -----<br>-----<br>0.025<br>0.00<br>0.004 | 0.025<br>0.00<br>0.004 |
| 60 | 2. Formaldehyde Solution, inhibited 12-15% methanol----- | 0.1222<br>0.1225<br>0.1290                     | -----<br>0.02                           | 0.01                                     | 0.005                  |
| 65 | 3. Ferric Sulfate, 1% by weight-----                     | 0.1811<br>0.1785<br>0.1574<br>0.1628<br>0.1565 | -----<br>0.214<br>0.272<br>0.055        | 0.007<br>0.007<br>0.007                  | 0.007<br>0.007         |

70 It will be seen that in the case of corrosion by ammonium nitrate solution, the protective coating including tin diffused in 2 mils of nickel-phosphorus coating produces substantially lower corrosion rates than when the nickel-phosphorus coating is only 1 mil thick. Likewise in the case of the formaldehyde solution and ferric sulfate solu-

tion, the 2 mils nickel-phosphorus coating treated with the diffusion tin process produces lower corrosion rates.

Other sources of tin can be utilized in the place of the stannous chloride utilized in the foregoing examples. Stannic chloride is a suitable source of tin for the reaction of the present invention although certain modifications must be made in the system 500 of FIG. 5 in order to utilize stannic chloride in place of stannous chloride. Whereas stannous chloride is a solid at room temperature and has an appreciable vapor pressure only in the temperature range 480° C. and up, stannic chloride is a liquid at room temperature and boils at approximately 113° C. In order to utilize stannic chloride in the system 500, ammonia gas is fed from the conduit 551 to the furnace 555 without heating thereof and is then swept across the stannic chloride which is maintained in the chamber 510 at room temperature. The nitrogen gas with the stannic chloride therein is fed through the line 513 to the tube 514. Simultaneously cracked ammonia is fed from the line 507 through the valve 519 and the line 516 to the tube 514, the precracked ammonia being maintained at an elevated temperature. The resultant mixture of nitrogen gas, stannic chloride vapors and cracked ammonia are then fed to the chamber 531 which is maintained at a suitable temperature such as 630° C. The reaction rate utilizing stannic chloride is comparable to that using stannous chloride and produces a tin-nickel-phosphorus coating which is attractive and comparable to or exceeds the qualities of the coating obtained using stannous chloride as a source of tin. The use of stannic chloride has the advantage over the use of stannous chloride that the furnace 512 need not be utilized when stannic chloride is utilized as the source of tin.

Other halides of tin may be utilized as the source of tin for carrying out the present process and more particularly stannous fluoride, stannous bromide and stannous iodide may be utilized as a source of tin.

#### EXAMPLE 9

The procedure of Example 1 was repeated utilizing stannous fluoride as the source of tin, the stannous fluoride being disposed in the chamber 510 and heated by the heater 512 to provide a substantial vapor pressure thereof whereby to mix a quantity of stannous fluoride vapors with the cracked ammonia gas. The reaction was carried out for a period of one hour at a temperature of 630° C. A satisfactory tin-nickel-phosphorus alloy layer was formed having properties comparable to those produced by the process of Example 1 above.

#### EXAMPLE 10

Workpieces were coated utilizing stannous bromide as a source of tin and precracked anhydrous ammonia gas as the reducing agent in the system 500 illustrated in FIG. 5. The heater 512 was operated to maintain the stannous bromide (B.P. 623° C.) at a temperature of approximately 480° C. The reaction was carried out at 630° C. for a period of one hour which produces on the workpieces 20 a gray coating having the desirable characteristics described above for tin-nickel-phosphorus alloy coatings.

#### EXAMPLE 11

A coating reaction was carried out utilizing the system 500 in FIG. 5 and employing stannous iodide (B.P. 720° C.) as a source of tin and precracked anhydrous ammonia gas as the reducing agent. The heater 512 was operated at 580° C. to supply sufficient stannous iodide vapors to provide the required amount of stannous chloride vapors on the reaction surface of the workpiece 20. The resulting tin-nickel-phosphorus coating had a bright metallic appearance, was uniform throughout, and possessed the desirable characteristics set forth above for such coatings.

The other stannic halides may also be used as a source of tin including stannic fluoride (sublimes at 705° C.), stannic bromide (B.P. 202° C.), and stannic iodide

(B.P. 340° C.), the temperature of the container 510 being adjusted to provide the suitable vapor pressure of the stannic halide therein.

In the preceding examples, the deposition of tin has been stated to have been upon nickel-phosphorus coatings produced by chemical nickel plating from plating baths of the nickel cation-hypophosphite type in which the nickel-phosphorus coating is utilized as plated. As plated, the nickel-phosphorus coating is an amorphous solid material consisting essentially of a metastable undercooled solution of phosphorus in nickel. The present process can also be applied to such nickel-phosphorus coatings which have been treated to form a nickel-phosphorus alloy, the method of producing the alloy from the amorphous solid material and the physical characteristics of the alloy being fully set forth in U.S. Patent No. 2,908,419 granted on October 13, 1959, to Paul Talmey and William J. Crehan. As is pointed out in the aforementioned Talmey and Crehan Patent No. 2,908,419, the character of the nickel-phosphorus coating is completely altered upon heat treatment to a critical temperature of about 400° C. whereby to convert the amorphous solid material to a stable solid material consisting essentially of micro-crystals of nickel-phosphide ( $Ni_3P$ ) dispersed in a matrix of nickel. The heat treatment is preferably carried out in an inert atmosphere such as nitrogen or in a reducing atmosphere such as cracked ammonia. The reaction is exothermic and proceeds with great rapidity throughout the nickel-phosphorus coating when the critical temperature is obtained. The heat treated nickel-phosphorus alloy has physical properties distinct from those of the nickel-phosphorus coating as chemically plated and more particularly the hardness of the alloy is substantially greater than the plating in that the nickel-phosphorus coating as plated has a hardness corresponding to V.H.N. of about 525, whereas the alloy may have a hardness corresponding to a V.H.N. of 950 or higher. In general the hardness of the alloy is greatest when heated at substantially the critical temperature of 400° C. and gradually decreases as the temperature of treatment increases so that the hardness after heat treatment at 630° C. would be from about V.H.N. 560 to 630.

The present processes can be readily applied to the heat treated nickel-phosphorus alloy whereby to produce the desired protective coating 31 comprising the tin-nickel-phosphorus alloy described heretofore. In those cases wherein the nickel-phosphorus coating is in the "as plated" condition and has not been heat treated, the nickel-phosphorus coating is in fact heat treated during the carrying out of the present process inasmuch as the workpiece 20 including the coating 22 is heated to 630° C., i.e., to a temperature well above the critical heat treatment temperature of 400° C. As a result, although the chemical nickel plated layer 22 may initially be an amorphous solid material consisting essentially of a metastable undercooled solution of phosphorus and nickel, upon treatment, the coating 22 is converted to a stable solid material consisting essentially of micro-crystals of nickel phosphide dispersed in a matrix of nickel and upon subjection of the coating 22 to a temperature of 630° C. for six hours would produce a hardness corresponding to a V.H.N. of about 575.

The present process is particularly suitable for treating hollow and tubular articles and there is shown in FIG. 8 of the drawings a system particularly adapted for treating a hollow article 820. The article 820 may be called a "container" or a "tank" and it is to be understood that these terms as employed herein are intended to cover all those hollow structures that perform a retaining, storing, conveying, etc., function and embrace a great variety of hollow structures commonly referred to as tubes, pipes, drums, barrels, etc. The container 820 has been illustrated as being made from two cylindrical sections 821 and 831 which are suitably joined together. More particularly the cylinder 821 is provided at one end

thereof with an outwardly directed flange 822 and at the other end thereof with a second outwardly directed flange 823, and the cylinder 831 is similarly provided at one end thereof with an outwardly directed flange 832 and at the other end thereof with a second outwardly directed flange 833. The flanges 823 and 833 are placed in abutting and contacting relationship and have aligned holes (not shown) formed therein to receive therethrough a plurality of bolts 838 having threaded outer ends receiving complementarily threaded nuts 839, whereby the bolts 838 and the nuts 839 serve to clamp the flanges 823 and 833 firmly against each other, a narrow crack or seam 837 being formed therebetween.

The container 820 has been shown mounted within an enclosure 801 including means to heat the contents thereof if desired whereby to permit coating of the internal surfaces of the container 820. More particularly, the container 820 is mounted upon two pairs of support rollers 808 and 809 that are respectively supported upon frames 810 and 811 by means of axles 812 and 813, respectively. A motor and gear box 815 has the output thereof connected to the shaft 812 whereby to drive the rollers 808 and thus to rotate the container 820 upon the rollers 808 and 809. Coating materials can be admitted to the interior of the container 820 from an inlet connection 802 passing through a rotary connection and seal 803 to a head or manifold diagrammatically illustrated at 804, the manifold 804 sealing the adjacent end of the container 820. The other end of the container 820 is provided with an outlet manifold 805 sealing the adjacent end of the container 820 and communicating with a rotary connection and seal 806 which in turn connects with an outlet 807.

In providing a protective coating upon the interior surfaces of the container 820 in accordance with the present process, the container is mounted as illustrated in FIG. 8 and a chemical nickel plating solution of the nickel cation-hypophosphite anion type described heretofore is pumped into the inlet connection 802 and thus into the interior of the container 820. The container 820 is continuously rotated as the plating solution is continuously flowed therethrough from the manifold 804 to the manifold 805 thereby to produce upon the interior surface of the container 820 a nickel-phosphorus coating 840. If the material of construction of the container 820 is catalytic to the chemical nickel plating reaction, the coating 840 can be directly made thereupon; if the material of construction of the container 820 is not catalytic to the chemical nickel plating reaction, then the surface thereof can be treated to implant thereon catalytic growth centers whereby to permit deposition of the nickel-phosphorus coating 840 thereon.

The nickel-phosphorus coating 840 is of one piece and provides a continuous liner for both sections 821 and 831 and serves to fill and cover the joint 837 therebetween. At this point in the process the coating 840 is an amorphous solid consisting essentially of metastable under-cooled solid solution of phosphorus and nickel and may comprise, for example, 92% nickel and 8% phosphorus by weight. It is possible at this point in the process to heat treat the coating 840, but it is more economical to proceed directly with the deposition of tin thereon whereby to achieve heat treating of the coating 840 during the tin diffusion process.

After having put the coating 840 in place upon the interior surface of the container 820, the furnace 801 is operated to raise the temperature of the contents thereof including the container 820 to the operating temperature of 630° C. for the tin deposition reaction. Simultaneously nitrogen or the reducing gas is connected to the input connection 802 whereby to purge the interior of the container 820 of all air, water vapor and the like. After a suitable purging time, for example, of one-half hour, and after the container 820 has reached the operating temperature of 630° C., a mixture of reducing gas and

a suitable compound of tin is introduced through the input connection 802, it being understood that this reaction mixture is the same as that produced in the conduit 514 in FIG. 5. The reaction gases, including, for example, stannous chloride and precracked anhydrous ammonia gas are continuously circulated through the container 820 and in contact with the coating 840 and the exhaust gases are removed through the outlet manifold 805 to the outlet 807. The reaction is carried out for a period of time such as six hours whereby to provide upon the nickel-phosphorus coating 840 another coating 841 which is the tin-nickel-phosphorus alloy designated by the numeral 31 in FIG. 4. The container 820 is heated for six hours while passing the reaction gases therethrough, and accordingly the typical three layer outer protective coating 31 of FIG. 4 is produced and simultaneously the nickel-phosphorus coating 22 is changed from an amorphous solid material to a stable solid material consisting of micro-crystals of nickel phosphide dispersed in a matrix of nickel. After formation of the protective coating 841, the container 820 is cooled in an inert or reducing atmosphere to a temperature of 200° C. after which it is removed from the furnace 801 and permitted to cool to the ambient temperature in the air. The resultant protective coating on the interior surface of the container 820 is continuous and of one piece and possesses the superior corrosion resistance properties discussed above with respect to the coating 31.

Referring now to FIGS. 9 to 11, inclusive, of the drawings, there is illustrated another form of a "container" or "tank," namely, a railway tank car 910 comprising mobile structure 911 carrying a shipping container or tank 912 embodying the features of the present invention. The tank 912, as illustrated, comprises a horizontally extending substantially cylindrical hollow body 913, two end headers 914, and a centrally disposed upstanding substantially cylindrical hollow dome 915. The body 913 includes a number of tubular sections 913a, five being illustrated, that are formed of steel plate and are secured by butt-welding at the meeting edges thereof to provide the seams or joints 916, as shown in FIG. 10; while the end headers 914 are also formed of steel plate and secured in lapped relationship by steel rivets 917 to the adjacent end sections 913a, as shown in FIG. 11. Further, the dome 915 is formed of steel plate and secured in a cooperating opening provided in the middle section 913a by arc welding, as indicated at 918. The construction of the tank 912, described above, and involving both welded and riveted joints between the various component elements thereof, is entirely conventional, and altogether arbitrary as a matter of structure, in order clearly to demonstrate the broad application of the present invention.

Continuing now with the construction of the tank 912, the dome 915 carries a removable steel cover 919, and the two end headers 914 are respectively provided with two steel fixtures 920 of tubular form, that, in turn, respectively carry two removable steel covers 921; which fixtures 920 may be employed in filling and in emptying the tank 912, when certain fluids are shipped or stored therein. Finally, the entire interior surfaces of the tank 912 are provided with a smooth continuous seamless liner 922, comprising a solid layer of nickel-phosphorus material intimately bonded to the interior surfaces mentioned. Also, the liner 922 completely covers the welded seams or joints 916 at the meeting edges of the sections 913a, as illustrated in FIG. 10, and the lapped edges of the end sections 913a and the end headers 914 at the riveted joints therebetween, together with the inner heads of the rivets 917, as illustrated in FIG. 11. Moreover, the liner 922 extends in covering relationship with the interior surfaces of the fixtures 920; whereby the liner 922 is of integral one piece construction throughout and is thoroughly devoid of cracks, seams or discontinuities of any kind whatsoever. Furthermore, the interior sur-

faces of the covers 919 and 921 are respectively provided with integral one piece liners, not shown, of the character of the liner 922; whereby the entire interior volume of the tank 912 is completely bounded by the one piece liner 922, and by the one piece liners, not shown, respectively carried by the interior surfaces of the covers 919 and 921.

The liner 922 may be applied in the same manner as the coating 840 described above and the liner 922 further has the surface thereof treated to diffuse tin thereinto to provide on the interior surface thereof a tin-nickel-phosphorus coating of the same character as the coating 841 described above with respect to FIG. 8.

In view of the foregoing, it will be appreciated that the coated workpieces 30 and 40 and the coated container 820 and the railway car 910 can be used in contact with a wide variety of fluids that cannot be permitted to have direct contact with the base metal 10 or the walls 821 and 831 of the container 820 and the car 910; whereby the range of utility of these workpieces and the container are greatly extended and are substantially wider than those attained by other types of protective coatings which have been employed heretofore and including such materials as rubber, glass, organic plastics, electrolytically deposited nickel, electrolytically deposited tin-nickel, chemically deposited nickel-phosphorus, etc., since it is obvious that many chemicals have selective corrosive or other deleterious actions on such materials aside from many other objectionable properties thereof. Also, it will be understood that the workpieces and container of the present invention are by no means limited to utilization in stationary chemical treatment or reaction apparatus but may be utilized in the fundamental transportation and distribution of such fluids, including corrosive reagents, and otherwise widely used in industry.

Also, the present process is particularly useful in imparting improved wearing qualities to work-pieces that are employed as bearing members; and there is shown in FIG. 12 of the drawings, a bearing bracket 1201 formed of steel, or the like, and carrying a bearing member 1202 embodying the features of the present invention. More particularly, the bearing member 1202 comprises a generally cylindrical support 1203 carrying a generally cylindrical liner 1204. The support 1203 is formed of a suitable base metal, such, for example, as steel or an aluminum alloy, while the liner 1204 comprises a nickel-phosphorus coating that is produced by chemical nickel plating from a plating bath of the nickel cation-hypophosphite anion type, as previously described. Further, the liner 1204 comprises a bearing surface 1204a that comprises the tin-nickel-phosphorus alloy that is produced by the present tin diffusion process. Accordingly, the liner 1204 comprises the outer portion of the nickel-phosphorus alloy plated upon the interior of the support 1203 and the inner portion providing the bearing surface 1204a and comprising the tin-nickel-phosphorus alloy as previously described. In the arrangement, the liner 1204 has a thickness of at least about 2 mils, as previously explained.

Finally, the bearing member 1202 supports a substantially cylindrical shaft 1205 in direct engagement with the bearing surface 1204a of the liner 1204, the shaft 1205 being formed of any suitable material and being mounted either for reciprocation or for rotation, as required in the mechanism in which the assembly as shown in FIG. 12 is incorporated.

As noted above, the bearing surface 1204a formed of the tin-nickel-phosphorus alloy possesses wearing qualities that are substantially superior to those possessed by the nickel-phosphorus alloy as produced directly by chemical nickel plating. In other words, the wearing qualities of the chemically plated nickel-phosphorus liner 1204 may be substantially improved by the present process, wherein the bearing surface 1204a of the liner 1204

is converted from a nickel-phosphorus alloy into a tin-nickel-phosphorus alloy.

This proposition will best be understood from an examination of certain comparative test data that were produced utilizing a conventional Amsler wear testing machine, as explained more fully below; and at this point, it is noted that the general principle of operation of the Amsler wear testing machine is diagrammatically illustrated in FIG. 13. More particularly, this machine comprises two substantially parallel arbors 1301 and 1302 that are rotated in the same direction. The arbor 1301 carries a tightly fitting standard specimen 1303 of generally cylindrical form, and the arbor 1302 carries a tightly fitting test specimen 1304 of generally cylindrical form. In turn, the test specimen 1304 comprises an inner test core 1304a of generally cylindrical form and an outer test coating 1304b of generally cylindrical form. In the arrangement, the arbors 1301 and 1302 are pressed toward each other and are rotated in the same direction, 10 the clockwise direction as indicated in FIG. 13; whereby the exterior surface of the standard specimen 1303 is disposed in frictional engagement with the exterior surface of the test coating 1304b of the test specimen 1304.

In the Amsler wear testing machine, gearing permits 25 one of the arbors 1301 to be directly driven, while the other of the arbors 1302 can be driven through a pendulum dynamometer, thereby to provide a continuous indication of the torque required to keep the two specimens 1303 and 1304 rotating at a constant speed. The torque 30 is recorded continuously and is integrated to give a measurement of the work required to move the two specimens 1303 and 1304 any given number of arbor revolutions.

In the present tests, the gearing mentioned was set so 35 that the arbor 1301 was rotated at 440 r.p.m., while the arbor 1302 was rotated at 400 r.p.m., whereby the test specimens 1303 and 1304 were operated under conditions of 110% slip in the engaging wearing surfaces thereof. Each of the specimens 1303 and 1304 had an external diameter of 2.352" and an axial length along the respective arbors 1301 and 1302 of 0.394"; whereby the wearing surfaces of the two specimens 1303 and 1304 were subjected to an equivalent speed of travel of about 512 ft. 40 per minute. The bearing load between the two arbors 1301 and 1302 was varied by the use of counterweights, and during these tests, the bearing loads ranged from 45 10# to somewhat in excess of 110#, as more fully explained hereinafter. The standard specimen 1303 was formed of 333-T5 aluminum alloy; the test core 1304a of the test specimen 1304 was formed either of steel or 50 333-T5 aluminum alloy; and the test coating 1304b was formed either of the nickel-phosphorus alloy as produced by chemical nickel plating or of the tin-nickel-phosphorus alloy as produced by the present process following the chemical nickel plating.

55 As explained more fully hereinafter, three of the tests were conducted in the presence of continuous lubricating oil between the contacting wearing surfaces of the specimens 1303 and 1304, while one of the tests was conducted in air after presoaking of the specimens 1303 and 1304 in lubricating oil. A light turbine oil was employed for the purpose mentioned having a viscosity of 50 305 Saybolt seconds at 100° F. and 50.8 Saybolt seconds at 210° F. Prior to each test, the specimens 1303 and 1304 were finished by circumferential grinding with a 60 Norton 38A120-JV abrasive wheel; and prior to testing, all specimens were cleaned by several washings in isopropyl alcohol and dried in a hot air blast.

In the tests, the specimens 1303 and 1304 were first 65 run at a bearing load of 10# for 24 hours in order to obtain "wearing-in," and thereafter the bearing loads were successively increased by 10# increments at each one-hour intervals until break-down or severe wearing of the specimens was produced. A continuous record 70 of the torque was made and measurements of the work 75

absorbed were made and the instantaneous or average coefficient of friction were calculated from these measurements. The data obtained were plotted as cumulative diameter loss and as an average coefficient of friction versus calculated bearing loads.

In a first of these tests, as illustrated in FIG. 14A, the standard specimen 1303 was formed of 333-T5 aluminum alloy; the test core 1304a was formed of steel, and the test coating 1304b was formed of nickel-phosphorus alloy, as obtained by chemical nickel plating. This first test was performed with continuous lubrication of the wearing surfaces of the specimens 1303 and 1304. The results of this first test are plotted graphically in FIG. 14A, wherein it is illustrated that the wear of the test specimen 1304 was somewhat greater than that of the standard specimen 1303. Moreover, in accordance with this test procedure, the threshold of substantial wear of both of the specimens was at about 68# of bearing load, and severe galling of both of the specimens occurred at 90# of bearing load.

In a second of these tests, as illustrated in FIG. 14B, the standard specimen 1303 was formed of 333-T5 aluminum alloy; the test core 1304a was formed of steel, and the test coating 1304b was formed of tin-nickel-phosphorus alloy, as produced by the present process following the chemical nickel plating. This second test was performed with continuous lubrication of the wearing surfaces of the specimens 1303 and 1304. The results of this second test are plotted graphically in FIG. 14B, wherein it is illustrated that the wear of the standard specimen 1303 was substantially greater than that of the test specimen 1304. Moreover, the threshold of some wear of the test specimen 1304 was at about 90# bearing load, and there was no severe galling in the test, although scoring of the specimens was initiated at a bearing load of approximately 100#.

By contrasting the results of the first test as plotted in FIG. 14A, with the results of the second test as plotted in FIG. 14B, it will be immediately appreciated that the tin-nickel-phosphorus alloy test coating 1304b has a vastly superior wear characteristic to that of the nickel-phosphorus alloy test coating 1304b; and it is emphasized that the tin-nickel-phosphorus alloy test coating 1304b was produced from the nickel-phosphorus test coating 1304b merely by the carrying out of the tin diffusion step of the present process.

In a third of these tests, as illustrated in FIG. 14C, the specimens 1303 and 1304 were identical to those employed in the second test, except that in this case, the tests were conducted in air after presoaking of the specimens 1303 and 1304 in the lubricating oil. The results of this third test are plotted graphically in FIG. 14C, wherein it is illustrated that the wear of the standard specimens 1303 was substantially greater than that of the test specimen 1304. Moreover, the threshold of some wear of the test specimen 1304 was at about 30# bearing load and there was no severe galling in the tests although scoring of the specimens was initiated at a bearing load of approximately 100#.

By contrasting the results of this third test, as plotted in FIG. 14C, with the results of the second test, as plotted in FIG. 14B, it will be immediately appreciated that the tin-nickel-phosphorus alloy of the test coating 1304b is admirably suited for use as a bearing surface in the absence of lubricating oil and under heavy load conditions during exceedingly long periods of time after it has once been soaked in lubricating oil. Not only does the tin-nickel-phosphorus alloy of the test coating 1304b exhibit the above-mentioned quality, but it also seems to effect lubrication of the standard specimen 1303 so as to prevent severe galling therebetween and notwithstanding the absence of continuous lubrication in this third test.

In a fourth of these tests, as illustrated in FIG. 15, the

standard specimen 1303 was formed of 333-T5 aluminum alloy; the test core 1304a was also formed of 333-T5 aluminum alloy, and the test coating 1304b was formed of a nickel-phosphorus alloy as obtained by chemical nickel plating. This fourth test was performed with continuous lubrication of the wearing surfaces of the specimens 1303 and 1304. The results of this fourth test are plotted graphically in FIG. 15, wherein it is illustrated that the wear of the standard specimen 1303 was somewhat greater than that of the test specimens 1304. Moreover, in accordance with this test procedure, the threshold of substantial wear of both of the specimens was at about 90# of bearing load and severe galling of both of the specimens occurred at 112# of bearing load.

By contrasting the results of the fourth test as plotted in FIG. 15, with the results of the first test as plotted in FIG. 14A, it will be immediately appreciated that the nickel-phosphorus alloy of the test coating 1304b is productive of better wearing qualities when it is applied to the test core 1304a formed of 333-T5 aluminum alloy than when it is applied to the test core 1304a formed of steel. This leads to the conclusion that the wearing characteristic of the test coating 1304b is related to the characteristic of the test core 1304a, and specifically that the softer test core 1304a formed of 333-T5 aluminum alloy is superior to the harder test core 1304a formed of steel as a mounting for the test coating 1304b.

In view of the foregoing, it will be apparent that a workpiece provided with the tin-nickel-phosphorus alloy coating is vastly superior as a bearing element to a workpiece provided with the nickel-phosphorus alloy coating; whereby it is highly advantageous to convert the nickel-phosphorus alloy coating of the tin-nickel-phosphorus alloy coating, utilizing the present process, when the workpiece is employed in service in which it is subjected to frictional contact with other elements or in which the workpiece is to serve as a bearing member.

While there has been described what is at present considered to be the preferred embodiment of the invention, it will be understood that various modifications may be made therein, and it is intended to cover in the appended claims all such modifications as fall within the true spirit and scope of the invention.

What is claimed is:

1. An article of manufacture comprising a base metal body carrying a coating of nickel-phosphorus intimately bonded thereto, said coating containing by weight about 85% to 97% nickel and about 3% to 15% phosphorus, the outer skin of said coating having tin diffused therein, said outer skin containing by weight about 1% to 50% tin and about 46% to 93% nickel and about 3% to 12% phosphorus.
2. The article of manufacture set forth in claim 1, wherein said coating has a thickness of at least about 2 mils.
3. An article of manufacture comprising a base metal body and a heat-hardened coating intimately bonded thereto, said coating comprising a nickel-phosphorus alloy containing by weight about 85% to 97% nickel and about 3% to 15% phosphorus, and the outer skin of said coating carrying substantial tin thermally diffuse therein, said outer skin containing by weight about 1% to 50% tin and about 46% to 93% nickel and about 3% to 12% phosphorus.
4. An article of manufacture comprising a base metal body carrying a coating of solid material intimately bonded thereto, said coating including an inner portion intimately bonded to said base metal body and an outer portion intimately bonded to said inner portion, said inner portion comprising a nickel-phosphorus alloy containing by weight about 85% to 97% nickel and about 3% to 15% phosphorus, said outer portion comprising a tin-nickel-phosphorus alloy containing by weight about 1% to 50% tin and about 46% to 93% nickel and about 3% to 12% phosphorus.

5. An article of manufacture comprising a base metal body carrying a coating of solid material intimately bonded thereto, said coating including an inner portion intimately bonded to said base metal body and an outer portion intimately bonded to said inner portion, said inner portion comprising a nickel-phosphorus alloy containing by weight about 85% to 97% nickel and about 3% to 15% phosphorus, said outer portion comprising a nickel-phosphorus alloy having tin diffused therethrough, said outer portion containing by weight about 1% to 50% tin and about 46% to 93% nickel and about 3% to 12% phosphorus.

6. An article of manufacture comprising a base metal body carrying a coating of solid material intimately bonded thereto, said coating including an inner portion intimately bonded to said base metal body and an outer portion intimately bonded to said inner portion, said inner portion comprising a heat-hardened nickel-phosphorus alloy containing by weight about 85% to 97% nickel and about 3% to 15% phosphorus and constituting a stable solid characterized by the presence of substantial micro-crystals of nickel phosphide disposed in a matrix of nickel, said outer portion comprising a heat-hardened nickel-phosphorus alloy having tin diffused therethrough, said outer portion containing by weight about 1% to 50% tin and about 46% to 93% nickel and about 3% to 12% phosphorus.

7. An article of manufacture comprising a base metal body carrying a coating of solid material intimately bonded thereto, said coating including an inner portion intimately bonded to said base metal body and an outer portion intimately bonded to said inner portion, said inner portion comprising a heat-hardened nickel-phosphorus alloy containing by weight about 85% to 97% nickel and about 3% to 15% phosphorus and constituting a stable solid characterized by the presence of substantial micro-crystals of nickel phosphide disposed in a matrix of nickel, said outer portion comprising a heat-hardened tin-nickel-phosphorus alloy containing by weight about 1% to 50% tin and about 46% to 93% nickel and about 3% to 12% phosphorus.

8. An article of manufacture comprising a base metal body carrying a coating of solid material intimately bonded thereto, said coating including an inner portion intimately bonded to said base metal body and an outer portion intimately bonded to said inner portion, said inner portion comprising a heat-hardened nickel-phosphorus alloy containing by weight about 85% to 97% nickel and about 3% to 15% phosphorus and constituting a stable solid characterized by the presence of substantial micro-crystals of nickel phosphide disposed in a matrix of nickel, said outer portion comprising three layers including a first layer intimately bonded to said inner portion and a second layer intimately bonded to said first layer and a third layer intimately bonded to said second layer, said first layer consisting essentially of tin distributed in said nickel-phosphorus alloy and containing by weight about 1% to 50% tin and the balance principally said nickel-phosphorus alloy, said second layer consisting essentially of said nickel-phosphorus alloy distributed in tin and containing by weight about 50% to 99% tin and the balance principally said nickel-phosphorus alloy, said third layer consisting essentially of tin.

9. An article of manufacture comprising a base metal body carrying a coating of solid material intimately bonded thereto, said coating including an inner portion intimately bonded to said base metal body and an outer portion intimately bonded to said inner portion, said inner portion comprising a heat-hardened nickel-phosphorus alloy containing by weight about 85% to 97% nickel and about 3% to 15% phosphorus and constituting a stable solid characterized by the presence of substantial micro-crystals of nickel phosphide disposed in a matrix of nickel, said outer portion comprising three layers including a first layer intimately bonded to said inner portion and a second layer intimately bonded to said first layer and a third

layer intimately bonded to said second layer, said first layer consisting essentially of tin distributed in said nickel-phosphorus alloy and containing by weight about 1% to 50% tin and the balance principally said nickel-phosphorus alloy, said second layer consisting essentially of said nickel-phosphorus alloy distributed in tin and containing by weight about 50% to 99% tin and the balance principally said nickel-phosphorus alloy, said third layer consisting essentially of tin, said coating having a hardness corresponding to at least V.H.N. 750.

10. A hollow container comprising a wall defined by one or more steel sheets securely joined together at the meeting edges thereof, a smooth continuous seamless and substantially homogeneous heat-hardened layer of solid material intimately bonded to the interior surfaces of both said one or more sheets and said one or more joints therebetween and in covering relationship therewith, the material of said layer comprising a nickel-phosphorus coating deposited from a plating bath of the nickel cation-hypophosphite anion type and containing by weight about 85% to 97% nickel and about 3% to 15% phosphorus, the outer skin of said nickel-phosphorus coating comprising a tin-nickel-phosphorus coating in which tin is diffused into said nickel-phosphorus coating and containing by weight about 1% to 50% tin and about 46% to 93% nickel and about 3% to 12% phosphorus, said tin-nickel-phosphorus coating also constituting a liner for said container and being also characterized by resistance to corrosive attack by ordinary acids, bases, and other reagents superior to that of electrodeposited nickel and that of said nickel-phosphorus coating.

11. A hollow container comprising a wall defined by one or more steel sheets securely joined together at the meeting edges thereof, a smooth continuous seamless and substantially homogeneous heat-hardened layer of solid material intimately bonded to the interior surfaces of both said one or more sheets and said one or more joints therebetween and in covering relationship therewith, the material of said layer comprising a nickel-phosphorus coating deposited from a plating bath of the nickel cation-hypophosphite anion type, said nickel-phosphorus coating being at least  $\frac{1}{2}$  mil thick and containing by weight about 85% to 97% nickel and about 3% to 15% phosphorus, the outer skin of said nickel-phosphorus coating comprising a tin-nickel-phosphorus coating in which tin is distributed in said nickel-phosphorus coating, said outer skin containing by weight about 1% to 50% tin and about 46% to 93% nickel and about 3% to 12% phosphorus, said tin-nickel-phosphorus coating also constituting a liner for said container and being also characterized by resistance to corrosive attack by ordinary acids, bases, and other reagents superior to that of electrodeposited nickel and that of said nickel-phosphorus coating.

12. A hollow container comprising a wall defined by one or more steel sheets securely joined together at the meeting edges thereof, a smooth continuous seamless and substantially homogeneous heat-hardened layer of solid material intimately bonded to the interior surfaces of both said one or more sheets and said one or more joints therebetween and in covering relationship therewith, the material of said layer comprising a nickel-phosphorus coating deposited from a plating bath of the nickel cation-hypophosphite anion type and constituting a stable solid characterized by the presence of substantial micro-crystals of nickel phosphide dispersed in a matrix of nickel and containing by weight about 85% to 97% nickel and about 3% to 15% phosphorus and having a resulting hardness within the approximate range 1000 V.H.N. to 575 V.H.N., the outer skin of said layer comprising a tin-nickel-phosphorus alloy containing by weight about 1% to 50% tin and about 46% to 93% nickel and about 3% to 12% phosphorus, said tin-nickel-phosphorus alloy also constituting a liner for said container and being also characterized by resistance to corrosive attack by ordinary acids, bases, and other reagents superior to that of elec-

trodeposited nickel and that of said nickel-phosphorus coating.

13. A tank formed of a base metal and having a liner of nickel-phosphorus alloy containing by weight about 85% to 97% nickel and about 3% to 15% phosphorus, the surface of said liner that is exposed to the contents of said tank having tin diffused therein and containing by weight about 1% to 50% tin and about 46% to 93% nickel and about 3% to 12% phosphorus.

14. A tank formed of a base metal and having a liner of nickel-phosphorus alloy containing by weight about 85% to 97% nickel and about 3% to 15% phosphorus, the surface of said liner that is exposed to the contents of said tank comprising a tin-nickel-phosphorus alloy containing by weight about 1% to 15% tin and about 46% to 93% nickel and about 3% to 12% phosphorus.

15. A bearing member formed of a base metal and provided with a bearing surface comprising a nickel-phosphorus alloy having tin diffused therein, said bearing surface containing by weight about 1% to 50% tin and about 46% to 93% nickel and about 3% to 12% phosphorus.

16. A bearing member formed of a base metal and provided with a bearing surface comprising a tin-nickel-

phosphorus alloy, said alloy containing by weight about 1% to 50% tin and about 46% to 93% nickel and about 3% to 12% phosphorus.

17. A bearing member comprising a base metal support carrying a liner formed essentially of a nickel-phosphorus alloy, containing by weight about 85% to 97% nickel and about 3% to 15% phosphorus, said liner being provided with a bearing surface having tin diffused therein and containing by weight about 1% to 50% tin and about 46% to 93% nickel and about 3% to 12% phosphorus.

18. The bearing member set forth in claim 17, wherein said support is formed essentially of steel.

19. The bearing member set forth in claim 17, wherein said support is formed essentially of aluminum.

20. The bearing member set forth in claim 17, wherein said liner has a thickness of at least about 2 mils.

References Cited in the file of this patent

UNITED STATES PATENTS

|           |               |               |
|-----------|---------------|---------------|
| 1,975,818 | Work          | Oct. 9, 1934  |
| 2,459,172 | Luetkekemeyer | Jan. 18, 1949 |
| 2,717,218 | Talmey        | Sept. 6, 1955 |
| 2,867,550 | Weber         | Jan. 6, 1959  |

UNITED STATES PATENT OFFICE  
CERTIFICATE OF CORRECTION

Patent No. 3,077,285

February 12, 1963

Pranas Budininkas

It is hereby certified that error appears in the above numbered patent requiring correction and that the said Letters Patent should read as corrected below.

Column 22, line 61, for "diffuse" read -- diffused --;  
column 23, line 26, after "12%" insert -- phosphorus --.

Signed and sealed this 3rd day of September 1963.

(SEAL)

Attest:

ERNEST W. SWIDER  
Attesting Officer

DAVID L. LADD  
Commissioner of Patents